

1

3,383,315

**POLYALKYLENE GLYCOL-DIORTHO SILICIC ACID ESTER LUBRICANTS AND POWER TRANSMITTING FLUIDS**

Herbert Göthel, Oberhausen-Sterkrade, Heinz Noeske, Oberhausen - Sterkrade - Nord, and Hans Feichtinger, Dinslaken, Germany, assignors to Ruhrchemie Aktiengesellschaft, Oberhausen-Holten, Germany, a corporation of Germany

No Drawing. Filed Aug. 31, 1965, Ser. No. 484,120

Claims priority, application Germany, Sept. 11, 1964,

R 38,770

10 Claims. (Cl. 252—49.6)

The present invention relates to novel diorthosilicic acid esters for use as additives to synthetic lubricants. Lubricants for turbine engines must meet certain standard specifications, which also serve as guide-lines for the development of synthetic lubricants.

For example, the British specification "Directionale of Engine Research and Development Material," Specif. vol., May 16, 1960, abbreviated "D-Eng. R.D.," 2487, specifies a minimum viscosity of 7.5 cst. at 98.9° C. for some lubricants. The synthetic ester oils heretofore employed in this respect are mixtures consisting of lubricating oil stocks and viscosity increasing additives. Di-basic esters of aliphatic alcohols and dicarboxylic acids possessing viscosities in the range of 3 to 4 cst. at 98.9° C. serve as lubricating oil stocks. Added thereto are complex ester additives or thickening agents with a viscosity of 10 cst. at 98.9° C. in adequate amounts in order to obtain mixtures with the required viscosity of 7.5 cst. at 98.9° C. (see Gunderson, Hart, "Synthetic Lubricants," Reichold P. Corp., New York, 1962, p. 197). These complex ester additives are prepared by reacting aliphatic alcohols and diols with dicarboxylic acids; their molecular weights range around 800. Other thickening agents are polyoxyalkylenes and polyglycols respectively.

The aging resistance and the high temperature characteristics of the above-mentioned additives are not completely satisfactory, especially under conditions prevailing in supersonic aircraft engines, in which high temperatures may occur in the bearings.

Heretofore, thickening agents could not be found, which were substantially satisfactory for these requirements. Thickening agents for mineral lubricating oils known in the art, as for instance polymethacrylates, improve the viscosity index of the basic oils, however, exhibit shearing stability that is too low, while highly viscous mineral oil products possess unsatisfactory low temperature characteristics.

It is therefore an object of this invention to overcome these and other difficulties encountered in the art and to provide thickening agents for lubricants, which meet the requirements of supersonic aircraft turbine engines. The thickening agents are not only required to exhibit an excellent viscosity-temperature relationship and favorable properties at extremely low temperatures, but must also be resistant to aging and possess adequate lubricity.

It has now been found that these objects may be accomplished by the novel polyoxyalkyleneglycol-diorthosilicic acid esters of the invention which have the following formula:



wherein R represents a polyoxyalkylene radical having

2

1 to 6, and preferably 2 to 4 ether oxygen atoms, each alkylene group comprising 2 to 4, preferably 2 or 3 carbon atoms, R represents a radical of a monoester (semi-ester) of a saturated straight-/or branched-chained carboxylic acid having 6 to 20 carbon atoms with an alkylene-/or oxyalkylene diol having 2 to 20 carbon atoms, R' represents an alkyl group having more than 3 carbon atoms, preferably up to 20 carbon atoms, and/or a polyoxyalkyleneglycol ether radical having 1 to 6 ether oxygen atoms, n has a value from 0 to 4, and wherein the substituents R and R' present in the molecule may be the same or different. In accordance with the invention, diorthosilicic acid esters of the formula:



wherein A, R and R' are as defined above constitute preferred diorthosilicic acid esters.

Depending on their viscosity, the esters of the invention are generally applied as thickening agents in amounts ranging from 5 to 70 volume percent and preferably from 25 to 70 volume percent, in regard to the quantity of the entire admixture. They can be admixed with other fluid bodies known in the art as lubricants, as for instance with mineral lubricating oils, dicarboxylic acid esters, phosphoric acid esters, organosilicium compounds of different structure; they are especially well suited as thickening agents for ester oils of the lubricating range. They do not only increase the viscosity of the basic oil stock, but also improve the viscosity index. Oxidation inhibitors known in the art, for instance phenothiazine and conventional effective substances may be added to the mixtures comprising the esters according to the invention.

The diorthosilicic acid esters of this invention were hitherto not yet described. They may be prepared by the conventional methods employed for the production of diorthosilicic acid esters as known in the art. The novel esters can be prepared, for instance, by reacting stoichiometric amounts of suitable starting materials with gaseous  $SiCl_4$  according to the disclosure of German Patent 1,142,855, or as disclosed in German patent application R 32,696, Auslegeschrift 1,180,359.

Especially suitable starting materials for the R-substituents are, for instance, carboxylic acid semiesters of ethyleneglycol, diethyleneglycol, triethyleneglycol, tetraethyleneglycol, propyleneglycol, polypropyleneglycol, 1,6-hexanediol and the like. The acid components of the said carboxylic acid semiesters may be prepared by the so-called oxo-synthesis, as for instance, trimethylhexanoic acid and other acids, which can be obtained by hydroformylation (oxo-synthesis) of medium and higher olefins, especially polyolefins, followed by air oxidation.

The properties of some "mixed" diorthosilicic acid esters, which can be applied according to the invention are set out in Table I which follows.

The esters of the invention listed in Table I are:

- I. Diethyleneglycol-di-orthosilicic acid - hexa-(diethyleneglycol-3,5,5-trimethylhexanoic acid ester)-ester,
- II. Triethyleneglycol-di-orthosilicic acid - hexa - (triethyleneglycol-3,5,5-trimethylhexanoic acid ester)-ester,
- III. Triethyleneglycol - di-orthosilicic acid-tri-(triethylen-

- glycol-3,5,5-trimethylhexanoic acid ester) - tri - (isodecyl)-ester,  
**IV.** Triethyleneglycol-di-orthosilicic acid-tri - (triethylene-glycol - 3,5,5 - trimethylhexanoic acid ester)-tri-(isotri-decyl)-ester,  
**V.** Triethyleneglycol-di-orthosilicic acid-tri - (triethylene-glycol - 3,5,5-trimethylhexanoic acid ester)-tri-(isoctadecyl)-ester,  
**VI.** Triethyleneglycol-di-orthosilicic acid-tri - (triethylene-glycol-3,5,5 - trimethylhexanoic acid ester)-tri-(diethylene-glycol-n-butylether)-ester,  
**VII.** Triethyleneglycol-di-orthosilicic acid-tri-(triethylene-glycol-3,5,5-trimethylhexanoic acid ester)-tri-(diethylene-glycol-ethyl-ether)-ester,  
**VIII.** Triethyleneglycol-di-orthosilicic acid - tri-(diethylene-glycol-3,5,5-trimethylhexanoic acid ester) - tri-(diethylene-glycol-n-butylether)-ester.

These esters are prepared in the so-called "bubble column reactor," according to the process disclosed in German patent application R 32,696, Auslegeschrift 1,180,- 20 359.

The properties of the esters according to the invention are in comparison with those of esters known in the art having equal R'-substituents, but possessing no semi-ester 25 substituents R, listed in the following Table II.

The known esters set out in Table II are:

- IIIb.** Triethyleneglycol-di - orthosilicic acid - hexa - (isodecyl)-ester,  
**IVb.** Triethyleneglycol-di-orthosilicic acid - hexa-(isotri-decyl)-ester,  
**Vb.** Triethyleneglycol-di-orthosilicic acid-hexa - (isoctadecyl)-ester,

as well as the following esters, which were heretofore proposed as lubricants:

- VIIb.** Triethyleneglycol-di-orthosilicic acid-hexa-(diethylene-glycol-n-butylether)-ester,  
**VIIib.** Triethyleneglycol-di-orthosilicic acid - tri - diethylene-glycol-n-butylether) - tri - (diethyleneglycol-ethyl-ether)-ester.

As is seen from a comparison of Tables I and II, the viscosity-temperature responsivity as well as the load carrying capacity of the esters according to the invention is influenced by the carboxylic acid ester radicals. Due to the substitution of these semi-ester radicals R in the molecule of the diorthosilicic acid esters their viscosity is considerably increased, except of ester V whose viscosity is somewhat lower than that of ester Vb, however, the viscosity index of ester V amounts to 127, while that of ester Vb is only 87.

If the ester molecule besides the carboxylic acid ester radicals additionally contains oxyalkyleneglycoether substituents, an increase of the viscosity and an improvement of the viscosity-temperature relationship results.

The load carrying capacity of the lubricating films of the several esters hereinbefore described was determined by means of the four-ball apparatus, as described by Boerlage (Lexikon der Schmiertechnik, G. Voegtle, Franck'sche Verlags-handlung Stuttgart, 1964). In Tables I and II, in the column "welding value," two values are given; the first number represents the highest load in kg. which the lubricating film being tested withstands for one minute without alteration, while the second number represents that load at which the balls are welded, i.e., frozen, together. The esters of the invention exhibit a better load carrying capacity than pure mineral oils and ester oils known in the art. The welding values of mineral oils amount to about 150/170 kg., those of dibasicester oils to 140/170 kg. The esters of the invention I to VIII possess—in comparison with esters IIIb to Vb—a more favorable load carrying capacity of the lubricating films formed thereof.

| No.  | A                                                                                                                    | R                                                                                                    | Polyoxyalkyleneglycol-diorthosilicic acid |                  |                              |                                       | Setting point, °C. | Welding value, load in kg. |
|------|----------------------------------------------------------------------------------------------------------------------|------------------------------------------------------------------------------------------------------|-------------------------------------------|------------------|------------------------------|---------------------------------------|--------------------|----------------------------|
|      |                                                                                                                      |                                                                                                      | n                                         | Molecular weight | d <sub>4</sub> <sup>20</sup> | Viscosity (est.) at 37.8° C. 38.9° C. |                    |                            |
| I    | —CH <sub>2</sub> CH <sub>2</sub> OCH <sub>2</sub> CH <sub>2</sub> —                                                  | (CH <sub>2</sub> CH <sub>2</sub> O) <sub>2</sub> COCH <sub>2</sub> CH(CH <sub>3</sub> ) <sub>3</sub> | —                                         | 1,630            | 1.039                        | 73.8 11.7                             | 138                | —50 170/190                |
| II   | —CH <sub>2</sub> CH <sub>2</sub> OCH <sub>2</sub> CH <sub>2</sub> OCH <sub>2</sub> CH <sub>2</sub> —                 | (CH <sub>2</sub> CH <sub>2</sub> O) <sub>3</sub> COCH <sub>2</sub> CH(CH <sub>3</sub> ) <sub>3</sub> | 0                                         | 1,938            | 1.067                        | 124 19.2                              | 140                | —48 180/190                |
| III  | —CH <sub>2</sub> CH <sub>2</sub> OCH <sub>2</sub> CH <sub>2</sub> OCH <sub>2</sub> CH <sub>2</sub> CH <sub>2</sub> — | (CH <sub>2</sub> CH <sub>2</sub> O) <sub>2</sub> COCH <sub>2</sub> CH(CH <sub>3</sub> ) <sub>3</sub> | —                                         | 1,542            | 1.006                        | 85.0 15.1                             | 147                | —45 170/180                |
| IV   | —CH <sub>2</sub> CH <sub>2</sub> OCH <sub>2</sub> CH <sub>2</sub> OCH <sub>2</sub> CH <sub>2</sub> CH <sub>2</sub> — | (CH <sub>2</sub> CH <sub>2</sub> O) <sub>3</sub> COCH <sub>2</sub> CH(CH <sub>3</sub> ) <sub>3</sub> | 3                                         | 1,695            | 1.032                        | 148 23.8                              | 141                | —49 170/180                |
| V    | —CH <sub>2</sub> CH <sub>2</sub> OCH <sub>2</sub> CH <sub>2</sub> OCH <sub>2</sub> CH <sub>2</sub> CH <sub>2</sub> — | (CH <sub>2</sub> CH <sub>2</sub> O) <sub>2</sub> COCH <sub>2</sub> CH(CH <sub>3</sub> ) <sub>3</sub> | 3                                         | 1,873            | 0.972                        | 142 17.5                              | 127                | —48 170/180                |
| VI   | —CH <sub>2</sub> CH <sub>2</sub> OCH <sub>2</sub> CH <sub>2</sub> OCH <sub>2</sub> CH <sub>2</sub> CH <sub>2</sub> — | (CH <sub>2</sub> CH <sub>2</sub> O) <sub>3</sub> COCH <sub>2</sub> CH(CH <sub>3</sub> ) <sub>3</sub> | 3                                         | 1,554            | 1.059                        | 90.0 124                              | 162                | —42 180/190                |
| VII  | —CH <sub>2</sub> CH <sub>2</sub> OCH <sub>2</sub> CH <sub>2</sub> OCH <sub>2</sub> CH <sub>2</sub> CH <sub>2</sub> — | (CH <sub>2</sub> CH <sub>2</sub> O) <sub>2</sub> COCH <sub>2</sub> CH(CH <sub>3</sub> ) <sub>3</sub> | 3                                         | 1,470            | 1.052                        | 820 21.0                              | 156                | —50 180/190                |
| VIII | —CH <sub>2</sub> CH <sub>2</sub> OCH <sub>2</sub> CH <sub>2</sub> OCH <sub>2</sub> CH <sub>2</sub> —                 | (CH <sub>2</sub> CH <sub>2</sub> O) <sub>3</sub> COCH <sub>2</sub> CH(CH <sub>3</sub> ) <sub>3</sub> | 3                                         | 1,422            | 1.072                        | 110 26.5                              | 151                | —48 170/180                |

TABLE II

| Diorthosilicic | Molec- | $d_4^{20}$ | viscosity (est.) at— | Viscosity index | Setting point, °C. | Welding value load |
|----------------|--------|------------|----------------------|-----------------|--------------------|--------------------|
| acid ester     | weight | 37.8° C.   | 98.9° C.             |                 |                    | in kg              |
| IIIb-----      | 1,146  | 0.923      | 34.6                 | 7.8             | 163                | 160/170            |
| IVb-----       | 1,398  | 0.905      | 56                   | 9.2             | 138                | 160/170            |
| Vb-----        | 1,818  | 0.897      | 740                  | 35.9            | 87                 | 150/160            |
| VIb-----       | 1,170  | 1.407      | 261                  | 7.0             | 189                | 180/190            |
| VIIb-----      | 1,086  | 1.067      | 24, 25               | 6.80            | 185                | 180/190            |

Due to the influence of their substituents, derived from high boiling substances, the esters according to the invention are substantially resistant to hydrolysis. They exhibit outstanding low temperature characteristics, which would aid starting turbine engines at low temperatures or temperatures encountered when flying at higher altitudes. The setting points set out in Table I depend on the high viscosity of the esters, which ranges above 180,000 cst., and are not caused by solid deposits. The silicic acid esters of the invention remain flowable under pressure. Their boiling points range above 440° C. at 760 mm. Hg and above 180° C. at 0.015 torr respectively. This high boiling range assures a low volatility. Due to the advantages mentioned hereinbefore, the esters of the invention are especially well suited as lubricants for turbo-jet engines.

Laboratory and test stand examination have indicated the oxidative and thermal stability of the compounds of the invention. The change of the viscosity and the acid content forms a criterion for oxidative and thermal stability. Since corrosion of the bearing metals may occur on increasing acid content of the lubricant, the corrosive influence of the lubricating components is determined by way of the changes in weight of metal test stripes simultaneously with the resistance against oxidation occurring at high temperatures, which is also catalyzed by metals, as for instance copper.

In Table III, which follows, the increase of the neutralization numbers (nN), the percentage change of the viscosity, the deposit of slurry, the changes in weight of copper-sheet stripes due to oxidation at high temperatures as well as the amount of split off-liquid products as volatility-test are listed for the esters I to VIII according to the invention.

The values of Table III were determined under aggravated testing conditions, exceeding those of corrosion-oxidation test standardized by specification D. Eng. R.D. 2487 of May 16, 1960, but using the same methods described therein. The latter are set in comparison with the testing conditions applied to the esters of the invention in Table IV, which follows.

15

TABLE IV.—CORROSION-OXIDATION TEST

|                                               | Testing conditions of Table III               |                                                                              |
|-----------------------------------------------|-----------------------------------------------|------------------------------------------------------------------------------|
| D. Eng. R. D. 2487                            | 140° C. $\pm 1^\circ$ C.                      | 200° C. $\pm 1^\circ$ C.                                                     |
| 140° C. $\pm 1^\circ$ C.                      | 22 h. $\pm 5$ min.                            | 32 h.                                                                        |
| 22 h. $\pm 5$ min.                            | Without passing through of air.               | Without passing through of air, 5 l./h.                                      |
| Without passing through of air.               | Change of the viscosity at 37.8° C.           | Change of the viscosity at 37.8° C.                                          |
| Change of the viscosity at 37.8° C.           | Max. $\pm 5\%$                                | See Table III.                                                               |
| Max. $\pm 5\%$                                | Increase of nN maximally up to 0.5 mg. KOH/g. | Increase of nN up to mg. KOH/g. (see Table III).                             |
| Increase of nN maximally up to 0.5 mg. KOH/g. | Change in weight of copper stripes.           | Change in weight of copper sheet stripes (258 $\pm 2$ mg./cm. <sup>2</sup> ) |
| Change in weight of copper stripes.           | See Table III.                                | cm. <sup>2</sup> = 40 sq. inch).                                             |

30 The substances to be tested were at first subjected to the conditions mentioned hereinbefore for 16 hours in absence of copper and thereafter for 16 hours in presence of the copper sheet strip. (The values set out in the tables were determined after 32 hours.)

35 One percent by weight phenothiazine (dispersible, Cassella Farbwerke Mainkur) was added as an oxidation inhibitor to 300 ml. of each of the substances to be tested.

40 The data obtained from the esters of the invention were compared with those of dibasic esters known in the art. The average values of bis-2-ethylhexylsebacic acid ester are listed under No. IX, those of some complex esters under No. X in Table III (identified in Gunderson, Hart, "Synthetic Lubricants," Reinhold P. Corp., New York, 1962, p. 197).

45 The comparison of the diorthosilicic acid esters according to the invention with the esters known in the art indicates that the esters of the invention exhibit higher oxidative stability. Their corrosivity determined at 200° C. on copper ranges below the limiting value of  $\pm 0.2$  mg./cm.<sup>2</sup> for the corrosion oxidation test at 140° C. according to D. Eng. R.D. 2487. Of considerable importance are the low slurry deposits or the slurry-carrying 50 capacity of the diorthosilicic acid esters of the invention.

55

TABLE III.—OXIDATIVE-STABILITY AND CORROSION TESTS

| Diorthosilicic acid ester | Increasing of the neutralization number on mg. KOH/g. | Change of the viscosity at 37.8° C. in percent | Deposit of slurry in percent | Change of weight of copper, mg./cm. <sup>2</sup> | Volatility test: amount of liquid products split-off in percent by vol. of the charge |
|---------------------------|-------------------------------------------------------|------------------------------------------------|------------------------------|--------------------------------------------------|---------------------------------------------------------------------------------------|
| I-----                    | 0.8                                                   | -4.4                                           | 0.36                         | -0.19                                            | 1.57                                                                                  |
| II-----                   | 0.8                                                   | -4.2                                           | 0.32                         | -0.19                                            | 1.50                                                                                  |
| III-----                  | 0.5                                                   | +4.0                                           | 0.56                         | -0.077                                           | 2.1                                                                                   |
| IV-----                   | 0.7                                                   | +6.4                                           | 0.6                          | -0.116                                           | 2.25                                                                                  |
| V-----                    | 0.8                                                   | +2.0                                           | 0.7                          | +0.155                                           | 1.9                                                                                   |
| VI-----                   | 0.8                                                   | -5.2                                           | 0.30                         | +0.116                                           | 1.9                                                                                   |
| VII-----                  | 0.4                                                   | -6.2                                           | 0.35                         | +0.116                                           | 2.13                                                                                  |
| VIII-----                 | 0.4                                                   | -5.5                                           | 0.32                         | +0.116                                           | 2.05                                                                                  |
| IX-----                   | 2.1-2.3                                               | +6.0                                           | 1.13                         | +0.039                                           | 2.1                                                                                   |
| X-----                    | 1.7-2.2                                               | +8.0-12.1                                      | (1)                          | +0.077-0.13                                      | 2.0-2.5                                                                               |

<sup>1</sup>Above 1.0.

Since high altitude flight requires engine oils exhibiting low volatility, due to the low pressures encountered under such conditions, the evaporation of the esters was tested under aggravated conditions (passing air through at 200° C.) simultaneously with their oxidative stability. The amount of the liquid products split-off from the esters of the invention is generally lower than that or equal to that respectively split-off from the known esters compared therewith.

The following examples are intended to illustrate the invention as certain embodiments thereof, and are not to be interpreted as limiting the same.

#### EXAMPLE I

A reaction vessel (a so-called bubble-column reactor) consisting of a vertical glass tube with an internal diameter of 69 mm. and a height of 550 mm. provided with a glass frit (Jena apparatus glass, grain coarseness 2) in its bottom, was charged with 107 g. triethyleneglycol, 347 g. diethyleneglycol-n-butylether and 622 g. triethyleneglycol-monoisononanate, which had previously been dried to a water content below 0.1 percent. Silicon tetrachloride was applied dropwise from a dosing vessel into an evaporator coil heated at 80° C., which was gastight connected with the said reaction vessel, by a conduit joining the said reaction vessel below the said glass frit. The silicon tetrachloride vapors evolved in the evaporator coil were sucked through the frit under a vacuum of 180 torr. The ascending  $\text{SiCl}_4$  vapors together with the hydrogen chloride evolved during the reaction formed a bubble-column of 420 mm. height with the liquid in the reactor. The liquid reaction mixture, which had been preheated to 40° was heated up to 52° C. by the heat of reaction. In order to compensate for the decreasing evolution of heat during the reaction, the reaction mixture was heated at about 50° C. during the course of the reaction. 221 g.  $\text{SiCl}_4$  were introduced and converted during 100 minutes. After termination of the reaction, the reaction vessel was heated at 110° C. for two hours, whereby dissolved hydrogen chloride was removed from the reaction mixture under introduction of nitrogen at a vacuum of 20 torr. (After the said treatment the Beilstein-reaction was negative.) Thereafter, the non-reacted excess amounts of the reactants (145 g.) were distilled off from the reaction product under a vacuum of 0.01 torr up to a temperature of 228° C. A distillation residue triethyleneglycol-diorthosilicic acid - tri-(diethyleneglycol-n-butylether)-tri-(diethyleneglycol-monoisononanate)-ester (ester VI of the invention) was obtained.

5 rator coil, which was gastight connected with the said reaction vessel by a conduit joining it below the said glass frit. The  $\text{SiCl}_4$  vapors were sucked through the glass frit under a vacuum of 180 torr into the reaction vessel.

5 The liquid mixture, preheated to 40° C. was heated at 56° C. by the reaction heat evolved in the bubble column formed in the reaction vessel by the ascending vapors of silicon tetrachloride and hydrogenchloride evolved during the reaction together with the liquid reactants. The reaction 10 was complete after 100 minutes. Hydrogen chloride dissolved in the reaction was removed at a vacuum of 18 torr under introduction of nitrogen from the reaction mixture heated to 110° C. (Thereafter, the Beilstein-reaction was negative.) The non-reacted excess liquid components 15 (112 g.) were distilled off at 0.01 torr under heating up to 193° C. As distillation residue 848 g. diethyleneglycol-diorthosilicic acid-tri-(diethyleneglycol-n-butylether)-tri-(diethyleneglycol-monoisononanate)-ester with the following properties were obtained: Density  $d_4^{20}=1.076$ ; refraction index  $n_{20}^D=1.4530$ ; viscosity at 98.9° C. 23.8 cst.; viscosity 20 at 37.8° C. 135 cst.; viscosity index=144; viscosity-temperature constant=0.824; setting point ranging at -50° C.; flame point 238° C.; silicon content 4.14 percent (calculated 4.07 percent).

25 In analogous manner other esters according to the invention may be prepared.

#### EXAMPLE III

30 80 parts by volume of diethyleneglycol-di-isonononanate were admixed with 20 parts by volume triethyleneglycol-diorthosilicic acid - tri-(diethyleneglycol-n-butylether)-tri-(ethyleneglycol-monoisononate)-ester (ester VI of the invention). The properties of the lubricant so obtained (hereinafter called admixture 80/20 percent by volume) 35 are shown in comparison with those of its starting components in Table V, which follows.

#### EXAMPLE IV

30 50 parts by volume of diethyleneglycol-di-isonononanate 40 were admixed with 50 parts by volume triethyleneglycol-diorthosilicic acid - tri-(diethyleneglycol-n-butylether)-tri-(diethyleneglycol-monoisononanate)-ester (ester VIII of the invention). The properties of the lubricant so obtained 45 (hereinafter called admixture 50/50 percent by volume) are also shown in comparison with those of its starting components in the following Table V.

TABLE V

|                                      | $d_4^{20}$ | Viscosity in cst. at— |          |         | Viscosity index | Setting point, °C. | Flame point, °C. | Welding value load in kg. |
|--------------------------------------|------------|-----------------------|----------|---------|-----------------|--------------------|------------------|---------------------------|
|                                      |            | 98.9° C.              | 37.8° C. | -40° C. |                 |                    |                  |                           |
| Diethyleneglycol-diisonononate       | 0.943      | 3.12                  | 11.8     | 3.800   | 147             | -65                | 215              | 150/160                   |
| Ester VI                             | 1.069      | 124                   | 590      | 260/400 | 162             | -43                | 251              | 180/190                   |
| Example III admixture 80/20% by vol. | 0.983      | 7.6                   | 34.73    | 11,800  | 158             | -65                | 228              | 160/170                   |
| Ester VIII                           | 1.072      | 26.5                  | 110      | 42,800  | 151             | -48                | 248              | 170/180                   |
| Example IV admixture 50/50% by vol.  | 1.007      | 8.02                  | 40.4     | 12,110  | 152             | -64                | 230              | 160/170                   |

silicic acid - tri-(diethyleneglycol-n-butylether)-tri-(triethyleneglycol-monoisononanate)-ester (VI) having a density  $d_4^{20}=1.069$  and a refraction index  $n_{20}^D=1.458$  was obtained. The silicon content of the product ester was determined to 3.72 percent (calculated 3.61 percent); the viscosity of the ester at 98.9° C. was 124 cst., at 37.8° C. 590 cst.; its viscosity index amounted to 162, its viscosity-temperature constant was 0.790, its flame point ranged at 254° C.

#### EXAMPLE II

A so-called "bubble-column" reaction vessel consisting of a vertical glass tube having an interior diameter of 63 mm. and a height of 480 mm. provided with a glass frit (Jena apparatus glass, coarseness 2) in its bottom, was charged with a mixture consisting of 66.5 g. diethyleneglycol, 300.5 g. diethyleneglycol-n-butylether and 463 g. diethyleneglycol-monoisononanate, which had previously been carefully dried. From a dosing vessel, 194 g. silicon tetrachloride was applied dropwise into an evapo-

60 Thus there has been described a novel composition and method for improving the viscosity, load bearing qualities, lubricity, corrosion resistance and volatility of composite lubricants by the addition of the diorthosilicic acid ester compounds of this invention to known lubricants. The novel compounds of this invention may also be used in applications such as power transmitting fluids, 65 dampening fluids, electrical insulating fluids and the like, which are known in the art. Additions of the esters in this respect may also vary from 5 to 70 percent by volume, especially 25 to 70 percent by volume.

70 Although the invention has been described with reference to certain preferred embodiments, it is not intended that the invention is to be limited thereby, and any modifications of the novel compound, composition and method are intended to be included in the broad scope 75 of the invention as embodied in the following claims.

What is claimed is:

1. A lubricating oil comprising 5 to 70 volume-percent of a diorthosilicic acid ester of the formula:



wherein A represents a polyoxalkylene radical having 1 to 6 ether oxygen atoms, each alkylene group comprising 2 to 4 carbon atoms, R represents a radical of a semi-ester of a saturated carboxylic acid selected from the group consisting of a straight-chained and branched-chained carboxylic acids having 6 to 20 carbon atoms with at least one member selected from the group consisting of alkylene and oxyalkylenediols having 2 to 30 carbon atoms, R' is selected from at least one member of the group consisting of alkyl groups having more than 3 carbon atoms and polyoxyalkyleneglycol ether radicals having 1 to 6 ether oxygen atoms, and n is of the class consisting of 1 to 4 and 0, and R and R' may be the same or different, and an ester lubricating oil.

2. A lubricating oil comprising a mixture of 5-70 volume percent of a diorthosilicic acid ester of the formula:



wherein A represents a polyoxalkylene radical having 1 to 6 ether oxygen atoms, each alkylene group comprising 2 to 4 carbon atoms, R represents a radical of a semi-ester of a saturated carboxylic acid selected from the group consisting of straight-chained and branched-chained carboxylic acids having 6 to 20 carbon atoms with at least one member selected from the group consisting of alkylene and oxyalkylenediols having 2 to 30 carbon atoms, R' is selected from at least one member of the group consisting of alkyl groups having more than 3 carbon atoms and polyoxyalkyleneglycol ether radicals having 1 to 6 ether oxygen atoms, and n is of the class consisting of 1 to 4 and 0, and R and R' may be the same or different, and 30 to 95% of a lubricating oil different from said diorthosilicic acid ester.

3. A lubricating oil comprising 5 to 70 volume percent of triethyleneglycol-diorthosilicic acid-hexa-(triethyl-

eneglycol-3,5,5-trimethylhexanoic acid ester)-ester and an ester lubricating oil.

4. A lubricating oil comprising 5 to 70 volume percent of triethyleneglycol-diorthosilicic acid-tri-(triethyleneglycol - 3,5,5 - trimethylhexanoic acid ester)-tri-(isodecyl)-ester and an ester lubricating oil.

5. A lubricating oil comprising 5 to 70 volume percent of triethyleneglycol-diorthosilicic acid-tri-(triethyleneglycol - 3,5,5 - trimethylhexanoic acid ester)-tri-(diethyleneglycol-n-butylether)-ether and an ester lubricating oil.

6. A lubricating oil comprising 5 to 70 volume percent of triethyleneglycol-diorthosilicic acid-tri-(diethyleneglycol - 3,5,5 - trimethylhexanoic acid ester)-tri-(diethyleneglycol-n-butylether)-ester and an ester lubricating oil.

7. A lubricating oil comprising 5 to 70 volume percent of diethyleneglycol-diorthosilicic acid-hexa-(diethyleneglycol - 3,5,5 - trimethylhexanoic acid ester)-ester and an ester lubricating oil.

8. A lubricating oil comprising 5 to 70 volume percent of triethyleneglycol-di-orthosilicic acid-tri-(triethyleneglycol - 3,5,5 - trimethylhexanoic acid ester)-tri-(isotridecyl)-ester and an ester lubricating oil.

9. A lubricating oil comprising 5 to 70 volume percent of triethyleneglycol-di-orthosilicic acid-tri-(triethyleneglycol - 3,5,5 - trimethylhexanoic acid ester)-tri-(isooctadecyl)-ester and an ester lubricating oil.

10. A lubricating oil comprising 5 to 70 volume percent of triethyleneglycol-di-orthosilicic acid-tri-(triethyleneglycol - 3,5,5 - trimethylhexanoic acid ester)-tri-(diethyleneglycolethyl-ether)-ester and an ester lubricating oil.

#### References Cited

##### UNITED STATES PATENTS

|    |           |         |           |       |            |
|----|-----------|---------|-----------|-------|------------|
| 35 | 2,724,698 | 11/1955 | Kittleson | ----- | 252—49.6   |
|    | 2,947,772 | 8/1960  | Eynon     | ----- | 252—49.6 X |
|    | 3,029,269 | 4/1962  | Abbott    | ----- | 252—49.6   |
|    | 3,118,841 | 1/1964  | Moreton   | ----- | 252—49.6   |
| 40 | 3,133,111 | 5/1964  | Wheeler   | ----- | 252—49.6   |

DANIEL E. WYMAN, Primary Examiner.

W. H. CANNON, Assistant Examiner.

UNITED STATES PATENT OFFICE  
CERTIFICATE OF CORRECTION

Patent No. 3,383,315

May 14, 1968

Herbert Gothen et al.

It is certified that error appears in the above identified patent and that said Letters Patent are hereby corrected as shown below:

Column 1, line 65, "R" should read -- A --. Column 2, line 4, "straight-/" should read -- straight- --; line 5, "alkylene-/" should read -- alkylene- --. Column 4, TABLE I, second column, line 6 thereof, "CH<sub>2</sub>CH<sub>2</sub>OCH<sub>3</sub>CH<sub>2</sub>OCH<sub>2</sub>CH<sub>2</sub>-" should read -- CH<sub>2</sub>CH<sub>2</sub>OCH<sub>2</sub>CH<sub>2</sub>OCH<sub>2</sub>CH<sub>2</sub> --; same TABLE I, fourth column, line 7 thereof, "(CH<sub>2</sub>CH<sub>2</sub>O)<sub>2</sub>-C<sub>2</sub>H<sub>5</sub>" should read -- (CH<sub>2</sub>CH<sub>2</sub>O)<sub>2</sub>-n-C<sub>2</sub>H<sub>5</sub> --. Columns 5 and 6, TABLE II, the first line comprising "acid ester" "weight", "37.8° C.", "98.9° C.", and "in kg" should be canceled and inserted above the line separating the actual TABLE from the headings; same TABLE II, fourth column, line 6 thereof, "24, 25" should read -- 24.25 --; same columns 5 and 6, footnote to TABLE III, "Above 1,0." should read -- Above 1.0. --. Column 6, line 45, "Reinhold" should read -- Reichold --. Column 9 line 11, cancel "a".

Signed and sealed this 9th day of December 1969.

(SEAL)

Attest:

EDWARD M. FLETCHER, JR.  
Attesting Officer

WILLIAM E. SCHUYLER, JR.  
Commissioner of Patents